

Aug. 8, 1933.

H. W. HALL

1,921,616

RACKET BOW

Filed June 5, 1931

2 Sheets-Sheet 1



Fig. 6.

Investor  
Horace W. Hall  
by Harold E. Cole  
attorney

Aug. 8, 1933.

H. W. HALL

1,921,616

RACKET BOW

Filed June 5, 1931

2 Sheets-Sheet 2



*Investor*  
Horace W. Hall  
by Harold E. Cole  
*Attorney*

## UNITED STATES PATENT OFFICE

1,921,616

## RACKET BOW

Horace W. Hall, Newton, Mass.

Application June 5, 1931. Serial No. 542,253

3 Claims. (Cl. 144—309)

This invention relates to tennis rackets and their manufacture, and particularly to a racket of relatively light weight.

There is considerable demand, especially by girls, for a racket of lighter than standard weight. Attempts to lighten a racket only an ounce or less have previously been unsuccessful because they were thereby materially weakened by reducing the thickness or depth of the bow. 10 In order to attain lightness manufacturers did the natural and obvious thing, that is, made the wooden bow thinner, with the result that they sacrificed strength to such an extent that light rackets were too fragile. In the development 15 of the present light racket I have proceeded in an entirely different manner, and have thereby attained lightness without material sacrifice of strength.

While my chief object has been to make a light, strong racket, an accompanying object was to produce one attractive in appearance. Still another object was to devise a new and economical method of manufacturing the wooden bow head and one whereby wooden laminations which have been steamed could be used 20 and still have strong glue joints.

The foregoing and other objects which will appear as the nature of the invention is better understood, may be accomplished by a construction, combination and arrangement of parts such as is disclosed by the drawings. The nature of the invention is such as to render it susceptible to various changes and modifications, and, therefore, I am not to be limited to the 30 methods and construction disclosed by the drawings and specification; but am entitled to all such changes therefrom as fall within the scope of my claims.

In the drawings:

40 Figure 1 is a perspective view showing a racket block bent around a caul with blotting paper between the wood laminations, partly broken away.

Figure 2 is a perspective view of a three-ply racket bow.

45 Figure 3 is a perspective view of a modified form of my invention showing a 5-ply racket bow.

Figure 4 is an enlarged section taken on the 50 line 4—4 of Figure 3 illustrating the 5-ply construction.

Figure 5 is an enlarged section taken on the line 5—5 of Figure 2 illustrating the 3-ply construction.

55 Figure 6 is a section taken on the line 6—6 of

Figure 1 illustrating the assembly of wood laminations and blotting paper between them.

As illustrated my tennis racket bow, which includes the head or curved portion and the straight handle portion, is formed of three wood 60 laminations, the two outside ones 12 being of a hard, heavy wood such as birch, and the inside or center lamination 13 being of a lighter wood such as spruce, all three of which are of such thickness as to require treatment, such as 65 steaming, before being bent to bow shape. This combination of relatively light and heavy woods has been arrived at after much study and testing, and it should be observed that the lighter, center lamination 13 is equal in thickness, or 70 slightly thicker, than said outside laminations 12. By thickness I refer to the actual thickness of the wood used, and which appears in and determines the width of the face of the racket, as indicated by the line T—T of Figure 3 of 75 the drawings. Heretofore it has been customary in a three-ply racket or any multi-ply racket of steamed wood laminations, to use a heavy, strong center ply which must necessarily be thinner than the outside plies because otherwise the weight of the bow would be excessive. 80

The wood for said inside lamination 13 should be stronger in proportion to its weight than the outside laminations 12, and this is true for instance of spruce as compared to birch. In 85 other words, I increase the thickness or face width of the bow over other rackets, and yet they are lighter and of sufficient strength.

In forming my bow I choose a wood such as birch, which is hard enough to withstand the 90 cutting tendencies of the string and is stiffer than ash, of approximately 5/32" thickness, for the outside laminations 12. For the inside lamination 13 I choose a wood such as spruce, which is much lighter than birch but 95 stronger in proportion to its weight, of a thickness of approximately 3/16". These laminations are sufficiently large so that about twelve racket bows may be cut out of one block, measuring roughly 63" x 10". They must be steamed 100 or otherwise treated to remove the internal stresses, and immediately after steaming and while in a saturated condition they are bent around a bow-shaped caul to the desired shape. I separate the laminations from each other 105 during this drying operation with a thin piece of blotting paper 15 or other absorbent material with the purpose in view of thoroughly drying, that is, absorbing the moisture on the outside surface of each lamination so that a strong glue 110

joint between them will be possible. The blotting paper absorbs the surface moisture as the wood is shaped, thereby thoroughly drying the surfaces of the laminations and making them 5 receptive to glue. It also prevents darker wood such as birch from discoloring a lighter wood such as spruce during the shaping process.

The surfaces of said laminations 12 and 13 which are to be joined together are covered 10 with a suitable adhesive, such as waterproof glue, and then said laminations are replaced upon said caul 14 and kept under pressure until the glue has set.

In the modification shown in Figure 3 of the 15 drawings I have inserted on each side of said center ply 13, so as to form a dark strip or line between it and each outer ply 12 a very thin lamination 16 of a dark wood such as walnut of approximately 1/32" in thickness. This walnut lamination 16 need not be steamed as it may be bent around said caul 14 in its natural condition. With this 5-ply construction said blotting paper 15 should be at least equal in thickness to said walnut lamination 16 so that during 20 the drying process said laminations 12 and 13 will be bent around the caul to a shape which will later accommodate said thin laminations 16 when they are glued and inserted between the other laminations. The center and outer laminations 13 and 12 respectively are, of course, 25 slightly thinner, when said walnut lamination 16 is used.

What I claim is:

1. A process in the manufacture of racket bows whereby laminations of wood are steamed, and immediately after steaming blotting paper placed between them and the whole bent around 80 a caul to the shape of a bow.

2. The process whereby a laminated racket bow is formed comprising steaming a plurality of wood laminations, placing thin sheets of absorbent material between them, bending said laminations and sheets around a caul to the 85 shape of a racket bow, then removing said sheets and applying glue to the surfaces of said laminations which were next to said sheets, then placing 90 said laminations together and then placing them on a caul and leaving them there until said glue has set.

3. A process in the manufacture of racket bows embodying steaming a plurality of wood laminations too thick to be bent to bow shape 95 without damaging internal strain, then inserting blotting paper between them and bending them to the shape of a racket bow, then removing said blotting paper and applying glue to the surfaces of said laminations whereby one may 100 be glued to another, then placing said laminations together, and then keeping them bent to the shape of a racket bow until said adhesive has set.

HORACE W. HALL. 105

35

110

40

115

45

120

50

125

55

130

60

135

65

140

70

145

75

150